

3,281,312

**FIBROUS PRODUCT CONTAINING RESINOUS MATERIAL AND POLYETHYLENE OXIDE AND PROCESS THEREOF**

Robert A. Fetters and Hanns F. Arledter, Chillicothe, Ohio, assignors to The Mead Corporation, Dayton, Ohio, a corporation of Ohio  
No Drawing. Filed Sept. 18, 1964, Ser. No. 397,599  
13 Claims. (Cl. 162—168)

This application is a continuation-in-part of Serial No. 121,821 filed July 5, 1961, now abandoned.

This invention relates to the production of evenly distributed resin in resin-filled fibrous material and, more particularly, to uniformly dispersed resin-filled moldable pulp material and products thereof.

It is recognized that the use of additives, such as various resins, in the making of paper is nearly as old as the making of paper. For example, rosin materials in small amounts have heretofore been added to paper fibers to size them against water penetration. Larger amounts of resinous materials have been added to plasticize paper. However, when the resinous material exceeds 4% of the paper-making pulp stock, desirable even distribution of the resinous material throughout the fibrous mass is not easily attainable commercially.

Numerous methods have been proposed in the patented art which attempt to obtain substantially even distribution of various resinous materials in fibrous webs. For example, cationic coupling agents have been proposed to adhere certain resins to fibers and the use of a cationic melamine as a fiber conditioning agent to flocculate impregnating resins has also been disclosed. However, such proposals present problems of critical control of process steps for producing resin-filled fibrous products where the resin is added to the fibers before forming into sheets or other desired shapes whereby the resin is uniformly dispersed throughout a formed mat.

The primary object of this invention is to provide a process for incorporating and substantially uniformly dispersing resinous materials in fibrous webs, which can be done easily and economically on existing papermaking equipment and without the need for critical control of process variables.

Another object is to provide a process for incorporating resinous materials in fibrous webs in which the resinous materials are substantially all retained and distributed substantially uniformly throughout the fibrous web.

A further object of the invention is to produce a resin-filled paper or board which may be easily formed under heat and pressure, and may be subsequently decorated by printing, painting, or lacquering.

A still further object is to produce a resin-filled fibrous product in which the physical properties of the fibrous product may be altered as desired by proper choice of resin, polyvalent metal salt, and pulp, and by the ratio of resin to pulp.

Another object is to provide a process of incorporating resinous materials in fibrous webs in which process problems such as slow drainage on the wire, plugging of the wire and felts, and sticking to the wire, felts, and dryer drums are substantially eliminated.

Other objects and advantages of this invention will become apparent from the following description and explanation of the invention.

This invention is predicated on the unexpected discovery and concept that the interaction of a polyvalent metal ion with a water or alkali soluble resinous material capable of being precipitated by a polyvalent metal ion, in intimate association with dispersed pulp fibers and the treatment of the resulting mixture with a dilute solution of a high molecular weight polyethylene oxide alone or in

combination with other additives will produce a substantially uniformly dispersed resin filled moldable material. As used herein, polyvalent means having a valence greater than unity.

5 In general, the process for carrying out this invention comprises: the treatment of dispersed pulp fibers with a polyvalent metal ion in the form of a salt, the treatment of the resulting pulp-metal ion mixture with water or alkali resinous material in solution and the treatment of the resulting mixture with a dilute solution of a high molecular weight polyethylene oxide.

High molecular weight polyethylene oxides of the type herein referred to which have been found to be preferable for use in this invention have molecular weights ranging from at least 1,000,000 to 10,000,000 and preferably of the order of 3,650,000 and are sold by Union Carbide Chemicals Company, Division of Union Carbide Corporation, under their generally identifying trademark Polyoxy. And by reason of innovations in catalysis as well as manufacturing techniques, these high molecular weight polyethylene oxide materials are available which have molecular weights ranging from about 50,000 to an excess of 10,000,000. Surprisingly, these high molecular weight materials are soluble in water and form relatively stable 10 solutions at temperatures below 100° C. Small amounts of these materials will thicken water so that it becomes a very viscous mass. As evidence of the extreme thickening properties of these particular high molecular weight polyethylene oxides, one such commercial product utilized by applicants has an average viscosity of 3,000 centipoises in a 1% aqueous solution. This particular material has a molecular weight of approximately 3,000,000. Another such commercial product has an average viscosity, as a 20 1% solution, of approximately 7,000 centipoises with its average molecular weight being about 6,000,000. Various techniques for producing the above type of polyethylene oxides are set forth in an article by F. N. Hill et al., entitled "High Molecular Weight Polymers of Ethylene Oxide," appearing at pages 5-7 of volume 50, No. 1, January 1958 issue of Industrial and Engineering Chemistry. Particular reference is made to the paragraph entitled "Polymerization" on page 7 of this article.

To facilitate the practice of this invention, the following general observations are submitted for carrying out the process so as to insure incorporating and substantially uniformly dispersing resinous materials in fibrous webs. The ingredients added in each process step should be thoroughly mixed before the next ingredient is added. Other than the time taken for thorough mixing, the reaction time taken for each step is not critical, providing at least several seconds are available for complete flocculation. Reasonable care should be exercised not to excessively agitate the stock after addition of the polyethylene oxide. Alternatively, the resin solution may be added to the pulp prior to the addition of the polyvalent metal ion which should be added to the pulp fibers in the form of a soluble salt, preferably a chloride salt, although certain nitrates, acetates and sulfates have been successfully used. Excessive amounts of polyvalent metal salts (up to three times the calculated stoichiometric amount needed) have been added without adversely affecting the process. Salts of the alkaline earth metals are preferred, although the following salts have been successfully used in the process: calcium chloride, aluminum sulfate (paper makers' alum), aluminum chloride, barium chloride, zinc sulfate, magnesium sulfate, beryllium nitrate, cadmium chloride, cobaltous chloride, cupric chloride, ferrous chloride, manganous chloride, mercuric acetate, nickelous chloride, stannic chloride, and strontium chloride. The salts may be added as finely divided solids, or in water solution.

Suitable resinous materials are reaction products of an

alkali hydroxide, such as sodium hydroxide, and a resinous acid or fatty acid or combinations of same. These reaction products are relatively water soluble and are used as aqueous solutions so that the resinous component will be intimately mixed with the pulp fibers.

The preferred resinous material is a mixture of the sodium salts of the acids present in tall oil and wood rosin, in a ratio of 85% tall oil and 15% rosin, hereinafter referred to as Resin A. Other materials are the sodium salts of wood rosin, tall oil fatty acids, extracted pine wood pitch, abietic, oleic, stearic, and linoleic acids, and mixtures of these acids used per se or after chemical modification. The ammonium salts of shellac and the sodium salts of alkali soluble polyvinyl acetate copolymers are also acceptable. The type of resinous material and polyvalent metal ion determine the melting point of the resinous component and to a considerable extent, the finished properties of the resin filled product.

The high molecular weight polyethylene oxide has been found to be particularly effective as a means of controlling the floc size of the precipitated resin metal salts, and in improving retention of same. Flocculating agents other than polyethylene oxide have been tried, but with limited success. The function of the polyethylene oxide appears to be one of controlled flocculation of the very fine precipitate formed by the reaction of the polyvalent metal ions with the resinous material. Furthermore, the polyethylene oxide appears to promote a high degree of uniform dispersion of the flocs in the fibrous mass. A range of from 0.002% to 0.1% of polyethylene oxide on resin-fiber content has been found to be effective in achieving this result, depending on the consistency of the stock. Best results have been obtained when the polyethylene oxide is added at the rate of 3.5 pounds of polyethylene oxide to 100,000 gallons of stock. The optimum amount of polyethylene oxide necessary for desired flocculation can be determined by simple observations. A sample of pulp stock containing precipitated resin taken after incorporating the flocculating agent shows a substantially clear water phase on settling if sufficient polyethylene oxide is present. Too much polyethylene oxide will cause the stock to appear slimy. A person skilled in the art can easily make these observations and adjust the amount of polyethylene oxide added. In general, stock which is highly agitated after addition of the flocculating agent, will require a higher percentage of flocculating agent. Corrections can easily and quickly be made by the operator during a paper machine run.

Small amounts of other materials may be added without departing from the scope of the invention. For example, in the formation of resin filled sheets, it is sometimes advantageous to add up to 0.4% of a melamine formaldehyde resin or polyethyleneimine (such as Kymene 557, a product sold by Hercules Powder Company), based on the resin-fiber content. Such addition may be made prior or following the addition of the flocculating agent. Defoamers may be added to control foam without materially affecting the process. Sulfuric acid and papermakers' alum have been added to control the pH of the resin filled sheet and resin properties.

It has been found that the temperature required to form or mold the resin-filled sheet of this invention can be adjusted by use of an acid or acid salt in combination with polyvalent metal ions. For example, addition of sulfuric

5 acid or papermakers' alum will reduce the temperature required to mold a paper board containing 20% of Resin A precipitated by calcium ion, the amount of molding temperature reduction amounting to about 20° F. Such adjustment of molding temperature greatly increases the 10 utility of the invention by adapting the product to existing molding presses of commerce. Such co-precipitation of the resin solution by acids or acid salts in combination with polyvalent metal ions presumably gives a mixed resin precipitate comprising free resin acid admixed with metal salts of the resin acid.

The process of this invention was developed primarily for use on paper or board machines. However, this process is readily applied to the preparation of resin filled pulp stock for making resin-pulp preforms and the like, as by 15 the usual pulp molding methods.

The invention will now be illustrated by the following examples which show specific embodiments thereof. However, it is to be understood that this invention in its broader aspects is not limited to these examples.

#### EXAMPLE 1

400 grams of double kraft liner corrugated cuttings were dispersed in 20,000 ml. of water in a conventional type disintegrator and blended for a period of at least 60 20 minutes. The pulp stock was then reduced to 1% consistency, and had a TAPPI freeness of 565 ml.

To 380 ml. portions of the 1% pulp stock were added 85 ml. of 3.0% Resin A solution, stirring the solution in slowly. Dilution water was added to give a subsequent 25 total volume of 790 ml. including all the desired additives. This corresponds to a resin-pulp consistency of 0.8%. Additional ingredients were added in the following manner. The calcium chloride was added as 35 ml. of a 0.1 molar water solution of  $\text{CaCl}_2$ . Kymene 557 was added as 6.35 ml. of a 0.1% water solution of Kymene 557. The polyethylene oxide was added as 3.15 ml. of 0.1% polyethylene oxide in water. After each addition the resin-pulp stock was thoroughly mixed, avoiding excessive agitation before the next ingredient was added.

30 Immediately after the desired ingredients had been thoroughly mixed, the resin-pulp stock containing the additives was poured into a British Sheet Machine filled with water up to the wire, and a handsheet was made without any further addition of water. The handsheet was then couched and dried. Several handsheets were made for each set of sheets, recording the time in seconds it takes to drain each sheet. Control sheets were made from the pulp stock without resin or other additives. All 35 sheets were dried to about 6% moisture at 220 to 245° F. The resin retention was calculated as follows:

$$\text{Percent Resin Retention} = (100)$$

Oven dry sheet weight — oven dry control sheet weight

Calculated dry resin weight added

40 The results for each set of sheets is given in Table I.

Table I

| Handsheet | Materials added to the pulp stock in the order of addition | pH   | Drainage time, sec. | Percent resin retention | White water |
|-----------|------------------------------------------------------------|------|---------------------|-------------------------|-------------|
| 1-A       | Resin A, only                                              | 8.33 | 1.3                 | 3.2                     | Dark,       |
| 1-B       | Resin A, $\text{CaCl}_2$                                   | 7.95 | 3.5                 | 76.4                    | Cloudy.     |
| 1-C       | Resin A, Kymene 557                                        | 8.65 | 1.8                 | 3.9                     | Dark.       |
| 1-D       | Resin A, Polyethylene oxide                                | 8.3  | 1.4                 | 8.8                     | Do.         |
| 1-E       | Resin A, $\text{CaCl}_2$ , Polyethylene oxide              | 8.3  | 2.6                 | 90.6                    | Clear.      |
| 1-F       | Resin A, Kymene 557, Polyethylene oxide                    | 8.7  | 1.7                 | 9.6                     | Dark.       |
| 1-G       | Resin A, $\text{CaCl}_2$ , Kymene 557, Polyethylene oxide  | 8.3  | 2.9                 | 92.8                    | Clear.      |
| 1-H       | Resin A, Kymene 557, $\text{CaCl}_2$ , Polyethylene oxide  | 8.4  | 3.1                 | 91.3                    | Do.         |

The handsheets of Example 1, as shown in Table 1, illustrate the synergistic effect of the polyvalent metal ion,  $\text{Ca}^{++}$ , and the polyethylene oxide on the retention of Resin A. In a comparison of Sheets 1-A containing no additives other than the resin, with Sheets 1-B, 1-C and 1-D, it can be seen that Kymene 557 had very little effect on resin retention, polyethylene oxide had only slightly better effect (+5.6%), and calcium chloride had a much greater effect (+73.2%). The combined additive effects of both calcium chloride and polyethylene oxide should be +78.8% whereas their synergistic effect demonstrated an actual increase of +87.3% resin retention as shown by Sheet 1-E. The lack of a synergistic effect between the polyethylene oxide and the Kymene 557 is

5  
10

indicate good drainage would be obtained on Fourdrinier or cylinder paper machines.

#### EXAMPLE 3

Using the pulp stock of Example 1, three sets of handsheets were made in which the 6.35 ml. of 0.1% water solution of Kymene 557 of Sheets 1-G reported in Table I were replaced with similar amounts of Parez 607, Amerex 8850, or polyethyleneimine. Parez 607 is a cationic melamine formaldehyde produced by American Cyanamid Company. Amerez 8850 is a liquid polyamide resin produced by American Marietta Company. The results for each of these sets of sheets is given in Table III.

Table III

| Handsheet  | Materials added to the stock and the order of addition            | pH  | Drainage time, sec. | Percent resin retention | White water   |
|------------|-------------------------------------------------------------------|-----|---------------------|-------------------------|---------------|
| III-A..... | Resin A, $\text{CaCl}_2$ , Parez 607, Polyethylene oxide.         | 8.1 | 2.8                 | 93.6                    | Almost clear. |
| III-B..... | Resin A, $\text{CaCl}_2$ , Amerez 8850, Polyethylene oxied.       | 8.3 | 3.2                 | 90.7                    | Clear.        |
| III-C..... | Resin A, $\text{CaCl}_2$ , Polyethyleneimine, Polyethylene oxide. | 7.8 | 2.9                 | 92.5                    | Do.           |

shown by Sheet 1-F, and is confirmed by Sheets 1-G and 1-H. The drainage times shown in the table indicate satisfactory drainage would be obtained in all cases on Fourdrinier or cylinder paper machines.

#### EXAMPLE 2

Using the pulp stock of Example 1, several sets of handsheets were made to demonstrate the effect of the order of addition on the retention of Resin A in the sheet.

The sheets were made using the procedure of Example 1, except that the order of addition of Resin A and other ingredients was changed, and the dilution water to make a subsequent total volume of 790 ml. was added to the pulp stock before the addition of the resin or other ingredients. The results for the sets of sheets for Example 2 are given in Table II.

35  
40  
45

All of the sheets showed good resin retention comparable to the results obtained with Sheets 1-G reported in Table I.

#### EXAMPLE 4

Using a 1% consistency pulp prepared from double kraft lined corrugated cuttings in the manner illustrated in Example 1, a series of handsheets was made to illustrate the effects of various polyvalent metal salts on the retention of Resin A with and without the addition of polyethylene oxide.

To a 380 ml. portion of the 1% pulp stock, enough dilution water was added to make a total volume of 790 ml. after the resin and other ingredients were added. To this, was added 85 ml. of 3.0% Resin A solution, stirring the solution in slowly. 35 ml. of a 0.1 molar water solution of polyvalent metal salt was then added, again with

Table II

| Handsheet | Materials added to the pulp stock in the order of addition | pH  | Drainage time, sec. | Percent resin retention | White water |
|-----------|------------------------------------------------------------|-----|---------------------|-------------------------|-------------|
| II-A..... | $\text{CaCl}_2$ , Resin A, Polyethylene oxide.             | 8.3 | 3.2                 | 92.0                    | Clear.      |
| II-B..... | $\text{CaCl}_2$ , Polyethylene oxide, Resin A.             | 8.3 | 2.9                 | 84.3                    | Cloudy.     |
| II-C..... | $\text{CaCl}_2$ , Resin A, Kymene 557, Polyethylene oxide. | 8.3 | 4.1                 | 90.1                    | Clear.      |
| II-D..... | $\text{CaCl}_2$ , Kymene 557, Resin A, Polyethylene oxide. | 8.2 | 3.3                 | 91.2                    | Do.         |
| II-E..... | Kymene 557, $\text{CaCl}_2$ , Resin A, Polyethylene oxide. | 8.3 | 3.2                 | 92.1                    | Do.         |
| II-F..... | Kymene 557, Resin A, $\text{CaCl}_2$ , Polyethylene oxide. | 8.3 | 2.6                 | 93.3                    | Do.         |

The handsheets as shown in Table II illustrate the effect of the order of addition of materials to the pulp stock. It is observed that if the polyethylene oxide is added last, as in the case of II-A and II-C though II-F, there is substantially no difference in retention of Resin A. However, adding the polyethylene oxide before the Resin A, as in Sheet II-B, reduced the resin retention, and the white water was cloudy, indicating the presence of precipitated resin in the white water. Drainage times again

70  
75

mild agitation, and 3.15 ml. of 0.1% polyethylene oxide in water was added, where indicated in Table IV. In the case of handsheet IV-DD (Table IV), 6.35 ml. of 0.1% Kymene 557 solution was also added following the addition of the aluminum sulfate.

The 0.1% polyethylene oxide was stirred in slowly, and a handsheet was made after mixing as described in Example 1. Several sheets were made for each variation. The results are recorded in Table IV.

Table IV

| Handsheet | Materials added to the stock and the order of addition                                     | pH  | Drainage time, sec. | Percent resin retention | Flocculation |
|-----------|--------------------------------------------------------------------------------------------|-----|---------------------|-------------------------|--------------|
| IV-A      | Resin A, BaCl <sub>2</sub>                                                                 | 7.6 | 2.5                 | 82.0                    | Fair.        |
| IV-B      | Resin A, BaCl <sub>2</sub> , Polyethylene oxide.                                           | 7.9 | 2.5                 | 96.4                    | Excellent.   |
| IV-C      | Resin A, ZnSO <sub>4</sub>                                                                 | 6.3 | 3.3                 | 45.1                    | Fair.        |
| IV-D      | Resin A, ZnSO <sub>4</sub> , Polyethylene oxide.                                           | 6.3 | 3.1                 | 62.9                    | Excellent.   |
| IV-E      | Resin A, MgSO <sub>4</sub>                                                                 | 8.0 | 4.0                 | 73.2                    | Fair.        |
| IV-F      | Resin A, MgSO <sub>4</sub> , Polyethylene oxide.                                           | 8.0 | 3.3                 | 89.0                    | Excellent.   |
| IV-G      | Resin A, CaCl <sub>2</sub>                                                                 | 6.5 | 2.2                 | 79.1                    | Fair.        |
| IV-H      | Resin A, CaCl <sub>2</sub> , Polyethylene oxide.                                           | 7.8 | 2.7                 | 91.6                    | Excellent.   |
| IV-I      | Resin A, Be(NO <sub>3</sub> ) <sub>2</sub>                                                 | 5.4 | 6.6                 | 91.3                    | Fair.        |
| IV-J      | Resin A, Be (NO <sub>3</sub> ) <sub>2</sub> , Polyethylene oxide.                          | 5.4 | 3.9                 | 94.5                    | Excellent.   |
| IV-K      | Resin A, CdCl <sub>2</sub>                                                                 | 6.3 | 2.7                 | 93.0                    | Fair.        |
| IV-L      | Resin A, CdCl <sub>2</sub> , Polyethylene oxide.                                           | 6.4 | 2.3                 | 98.6                    | Excellent.   |
| IV-M      | Resin A, CoCl <sub>2</sub>                                                                 | 6.9 | 4.0                 | 87.0                    | Fair.        |
| IV-N      | Resin A, CoCl <sub>2</sub> , Polyethylene oxide.                                           | 7.2 | 3.4                 | 94.2                    | Excellent.   |
| IV-O      | Resin A, CuCl <sub>2</sub>                                                                 | 5.4 | 7.5                 | 93.4                    | Good.        |
| IV-P      | Resin A, CuCl <sub>2</sub> , Polyethylene oxide.                                           | 5.4 | 4.9                 | 100.5                   | Do.          |
| IV-Q      | Resin A, FeCl <sub>2</sub>                                                                 | 6.4 | 6.2                 | 85.3                    | Fair.        |
| IV-R      | Resin A, FeCl <sub>2</sub> , Polyethylene oxide.                                           | 6.4 | 6.4                 | 89.7                    | Good.        |
| IV-S      | Resin A, MnCl <sub>2</sub>                                                                 | 7.1 | 3.6                 | 78.3                    | Fair.        |
| IV-T      | Resin A, MnCl <sub>2</sub> , Polyethylene oxide.                                           | 7.2 | 3.0                 | 91.8                    | Good.        |
| IV-U      | Resin A, Hg (Ac) <sub>2</sub>                                                              | 4.9 | 8.4                 | 84.7                    | Fair.        |
| IV-V      | Resin A, Hg (Ac) <sub>2</sub> , Polyethylene oxide.                                        | 4.6 | 4.0                 | 98.6                    | Excellent.   |
| IV-W      | Resin A, NiCl <sub>2</sub>                                                                 | 7.1 | 5.6                 | 86.1                    | Good.        |
| IV-X      | Resin A, NiCl <sub>2</sub> , Polyethylene oxide.                                           | 7.1 | 3.8                 | 94.1                    | Excellent.   |
| IV-Y      | Resin A, SnCl <sub>4</sub>                                                                 | 1.9 | 3.7                 | 75.9                    | Fair.        |
| IV-Z      | Resin A, SnCl <sub>4</sub> , Polyethylene oxide.                                           | 1.6 | 3.7                 | 96.5                    | Excellent.   |
| IV-AA     | Resin A, SrCl <sub>2</sub>                                                                 | 7.9 | 2.9                 | 71.1                    | Fair.        |
| IV-BB     | Resin A, SrCl <sub>2</sub> , Polyethylene oxide.                                           | 7.9 | 2.7                 | 85.6                    | Excellent.   |
| IV-CC     | Resin A, Al <sub>2</sub> (SO <sub>4</sub> ) <sub>3</sub>                                   | 3.8 | 16.4                | 82.9                    | Fair.        |
| IV-DD     | Resin A, Al <sub>2</sub> (SO <sub>4</sub> ) <sub>3</sub> , Kymene 557, Polyethylene oxide. | 3.8 | 4.4                 | 91.7                    | Excellent.   |

In this series of handsheets the degree of flocculations was determined by observations of the flocs and clarity of the water phase. In each case, the polyethylene oxide substantially increased the retention of the Resin A, and in most cases the drainage time was decreased by the addition of the polyethylene oxide.

#### EXAMPLE 5

A paste of sodium oleate was prepared in the laboratory by heating 100 grams of oleic acid with 20 grams of sodium hydroxide in enough water to make a total batch weight of 500 grams. The reacted paste was then dissolved in water and diluted to 3.56% solids. A portion of this solution was reacted with calcium chloride and this mixture was dried and the Parr Bar stick point was determined on the dried resin.

To a 380 ml. portion of the pulp stock of Example 4, enough dilution water was added to make a total volume of 790 ml. after addition of the resin and other ingredients. To this was added 71.5 ml. of 3.56% sodium oleate, 34.5 ml. of 0.1 molar calcium chloride, and 3.15 ml. of a 0.1% solution of polyethylene oxide in water. Between each addition, the resin pulp stock was thoroughly mixed before the addition of the next ingredient. A handsheet was made in the manner described in Example 1 and the data obtained are reported in Table V.

#### EXAMPLE 6

The procedure of Example 5 was repeated using 100 grams of abietic acid and 20 grams of sodium hydroxide.

#### EXAMPLE 7

The procedure of Example 5 was repeated using 50 grams of abietic acid, 50 grams of oleic acid and 20 grams of sodium hydroxide.

#### EXAMPLE 8

The procedure of Example 5 was repeated using 100 grams of linoleic acid and 20 grams of sodium hydroxide.

#### EXAMPLE 9

40 A paste of sodium palmitate was prepared in the laboratory by heating 100 grams of palmitic acid with 17.1 grams of sodium hydroxide in enough water to make a total batch weight of 500 grams. The reacted paste was then dissolved in water and diluted to 3.90% solids. A portion of this solution was reacted with calcium chloride and this mixture was dried and the Parr Bar stick point was determined on the dried resin.

45 To a 380 ml. portion of the pulp stock of Example 4, enough dilution water was added to make a total volume of 790 ml. after addition of the resin and other ingredients. To this was added 65 ml. of 3.90% sodium palmitate, 50 ml. of 0.1 molar calcium chloride and 3.15 ml. of a 0.1% solution of polyethylene oxide in water. Between additions, the stock was thoroughly mixed before the addition of the next ingredient. A handsheet was made 55 in the manner described in Example 1 and the data obtained are reported in Table V.

#### EXAMPLE 10

60 The procedure of Example 9 was repeated using 100 grams of K wood rosin and 14.63 grams of sodium hydroxide.

#### EXAMPLE 11

65 The procedure of Example 9 was repeated using 100 grams of WW wood rosin and 14.63 grams of sodium hydroxide.

#### EXAMPLE 12

70 The procedure of Example 9 was repeated using 100 grams of a distilled tall oil fatty acid containing 5% rosin acids, and 15.14 grams of sodium hydroxide.

#### EXAMPLE 13

75 The procedure of Example 9 was repeated using 100 grams of stearic acid and 14.06 grams of sodium hydroxide.

**9**  
**EXAMPLE 14**

100 grams of a commercial grade of alkali soluble vinylacetate copolymer were added to a solution of 5.5 grams of sodium hydroxide in 900 grams of water. The mixture was stirred until the vinylacetate copolymer was dissolved, diluted with water to approximately 3% solids, and the diluted solution was used in preparing and making handsheets.

To a 380 ml. portion of the pulp stock of Example 4, enough dilution water was added to make a total volume of 790 ml. after the addition of resin and the other ingredients. To this was added 86 ml. of 3% solution of polyvinyl acetate copolymer prepared above, 50 ml. of 0.1 molar aluminum chloride, and 3.15 ml. of a 0.1% solution of polyethylene oxide in water. Between additions, the stock was thoroughly mixed before the addition of the next ingredient. A handsheet was made in the manner described in Example 1 and the data obtained are reported in Table V.

**EXAMPLE 15**

50 grams of an orange shellac were added to 450 grams of water, and 5 grams of 28% ammonium hydroxide were then added to the mixture. This mixture was heated to 140° F. for 10 minutes, and the reacted resin, hereinafter referred to as Resin B, was cooled and diluted with water to approximately 3% solids.

To a 380 ml. portion of the pulp stock of Example 4, enough dilution water was added to make a total volume of 790 ml. after the addition of the resin and the other ingredients. To this was added 86 ml. of 2.96% solution of Resin B prepared as above, 100 ml. of 0.1 molar calcium chloride, and 3.15 ml. of a 0.1% solution of polyethylene oxide in water. Between additions, the stock was thoroughly mixed before the addition of the next ingredient. A handsheet was made in the manner described in Example 1.

**EXAMPLE 16**

150 grams of pulverized extracted pine wood pitch were dispersed in 375 grams of water containing 20 grams of sodium hydroxide. This mixture was stirred for 30 minutes, and the reacted resin, hereinafter referred to as Resin C, was diluted with water to approximately 3% solids.

To a 400 ml. portion of a .97% consistency slurry of double kraft lined corrugated cuttings having a TAPPI freeness of 565 ml. was added 84 ml. of 3% solution of Resin C following with 40 ml. of 0.1 molar calcium chloride. The pH of this mixture was adjusted to 5.0 by adding dilute sulfuric acid. Successive additions of 6.35 ml. of 0.1% Parez 607 and 3.15 ml. of a 0.1% solution of polyethylene oxide in water were made, and enough water was added to bring the total volume to 790 ml. The resin-fiber stock was then mixed thoroughly and a handsheet was made in the manner described in Example 1.

*Table V*

| Example No. | Resin                                        | pH  | Drainage time, sec. | Percent resin retention | Parr Bar stick point °F. |
|-------------|----------------------------------------------|-----|---------------------|-------------------------|--------------------------|
| 5-----      | Sodium Oleate-----                           | 9.6 | 4.0                 | 84.1                    | 188                      |
| 6-----      | Sodium Abietate-----                         | 9.6 | 5.0                 | 72.6                    | (*)                      |
| 7-----      | 50-50 Sodium Abietate-Sodium Oleate Mixture. | 9.8 | 5.5                 | 89.6                    | 277                      |
| 8-----      | Sodium Linoleate-----                        | 9.6 | 6.0                 | 89.5                    | 198                      |
| 9-----      | Sodium Palmitate-----                        | 8.1 | 4.6                 | 86.6                    | 310                      |
| 10-----     | Sodium Salt of K Wood Rosin-----             | 8.5 | 5.7                 | 81.4                    | 463                      |
| 11-----     | Sodium Salt of WW Wood Rosin-----            | 8.6 | 5.4                 | 85.5                    | 434                      |
| 12-----     | Sodium Salt of Tall Oil Fatty Acid-----      | 7.2 | 5.0                 | 82.0                    | 201                      |
| 13-----     | Sodium Stearate-----                         | 8.1 | 4.4                 | 92.7                    | 316                      |
| 14-----     | Alkali soluble vinylacetate copolymer.       | 4.3 | 3.7                 | 93.0                    | 450+                     |
| 15-----     | Resin B-----                                 | 8.2 | 45.7                | 88.3                    | (*)                      |
| 16-----     | Resin C-----                                 | 5.0 | 8.0                 | 84.1                    | (*)                      |

\*Not determined.

**10**  
**EXAMPLE 17**

To prepare a 40% resin-60% fiber board, 3400 grams of double kraft lined corrugated cuttings were furnished to a beater and beaten to a TAPPI freeness of 575 ml. The pulp stock was then dropped to a chest, and 1338 grams of dry Resin A and 935 grams of dry sodium salt of B wood rosin were added to the stock as dilute water solutions. Additional water was added to the resin-fiber stock in the chest to give a resin-pulp consistency of 0.8%.

10 400 grams of calcium chloride (dry basis) were dissolved in a minimum of water and added to the resin-fiber stock. This was added slowly while agitating the stock to insure complete and uniform resin precipitation. To this was added 700 ml. of 10% sulfuric acid and 94.5 ml. of 6% water solution of Parez 607, and thoroughly mixed. 284 ml. of a 1% water solution of polyethylene oxide was added, and the stock was mixed using a minimum of agitation. The pH of the stock was 5.4.

15 Using this stock, a resin-fiber board having a basis weight of 68 pounds per thousand square feet was produced on a Fourdrinier machine at a speed of 1.95 feet per minute. Due to agitation of the resin-pulp stock in the chest, a small amount of 1% polyethylene oxide was added as the trial progressed to insure good flocculation. 20 Formation and drainage of the sheet on the wire were good. The percent resin retention was calculated as follows:

Percent Resin retention =

$$30 \quad 100 - \left( \frac{\text{Filterable dry solids in white water}}{\text{Filterable dry solids in treated stock}} \right) \times 100$$

The calculated resin retention was 99.8%.

**EXAMPLE 18**

35 To prepare a 40% resin-60% fiber board, 3400 grams of double kraft lined cuttings were furnished to a beater and beaten to a TAPPI freeness of slightly over 500 ml. The pulp stock was dropped to a chest, and 1265 grams of dry Resin A and 885 grams of dry sodium salt of B wood rosin were added to the stock as dilute water solutions. Additional water was added to the resin-fiber stock to give a resin-pulp consistency of 0.8%.

40 323 grams of calcium chloride (dry basis) dissolved in a minimum amount of water were added to the diluted resin-pulp stock. The stock was thoroughly mixed, and 278 ml. of 1% polyethylene oxide in water were added. The stock was then mixed using a minimum of agitation. The pH of the treated stock was 7.1. Using this stock, a resin fiber board having a basis weight of 83 pounds per thousand square feet was produced on a Fourdrinier machine at a speed of 2.37 feet per minute. As in Example 18, flocculation was controlled in the chest by addition of small amounts of 1% polyethylene oxide during the trial. Formation and drainage of the sheet on the wire were good, and there was no evidence of plugging the wire or felts or sticking to the press or felts. The 45 calculated resin retention was 98.9%.

## EXAMPLE 19

To prepare a 25.8% resin-74.2% fiber board, 3400 grams of double kraft lined cuttings were furnished to a beater and beaten to a TAPPI freeness of slightly over 500 ml. The pulp stock was dropped to a chest, and 695 grams of dry Resin A and 485 grams of dry sodium salt of B wood rosin were added to the stock as dilute water solutions. Additional water was added to the resin-pulp stock to give a resin-pulp consistency of 0.8%.

332 grams of dry barium chloride were dissolved in a minimum amount of water and added to the resin-pulp stock. The stock was thoroughly mixed, and 229 ml. of 1% polyethylene oxide in water were added. The stock was mixed using a minimum of agitation. The pH of the stock was 7.05.

Using this stock, a resin fiber board having a basis weight of 83 pounds per thousand square feet was produced on a Fourdrinier paper machine without difficulty at a speed of 2.37 feet per minute. As in Example 18, flocculation was controlled in the chest by the addition of small amounts of 1% polyethylene oxide during the trial. Formation and drainage of the sheet on the wire were good, and there was no evidence of plugging the wire or felts or sticking to the press or felts. The calculated resin retention was 99.9%.

## EXAMPLE 20

To prepare a 46.8%-53.2% fiber board, 3240 grams of double kraft lined cuttings were furnished to a beater and beaten to a TAPPI freeness of 562. The pulp stock was then dropped to a chest, and 2812 grams of dry Resin A were added as a dilute water solution. Additional water was added to the resin-fiber stock in the chest to give a resin-pulp consistency of 0.8%.

To this stock was added successively, 422 grams of calcium chloride (dry basis) dissolved in a minimum of water, and 6.052 grams of Kymene 557 dissolved in 1212 ml. of water, mixing thoroughly between the addition of each ingredient. 606 ml. 0.5% polyethylene oxide in water was added, and the stock was mixed using a minimum of agitation. The pH of the stock was 5.5.

Using this stock, a resin fiber board having a basis weight of 83 pounds per thousand square feet was produced on a Fourdrinier paper machine at a speed of 4.0 feet per minute. As in Example 18, flocculation was controlled in the chest by the addition of small amounts of 0.5% polyethylene oxide during the trial. Formation and drainage of the sheet on the wire were good, and there were no evidences of plugging the wire or felts or sticking to the press or felts. The calculated resin retention was 98.5%.

## EXAMPLE 21

3550 pounds of double kraft lined corrugated cuttings were beaten in a hydropulper, at a stock consistency of about 4%, to remove large lumps of fibers. The TAPPI freeness of the resultant pulp was 430 ml. 200 pounds of a 76% commercial grade of calcium chloride were added to the hydropulper near the end of the beating cycle. After dewatering and dropping the stock to the beater chest, it was refined through the jordans, at a consistency of 4.45% to a TAPPI freeness of 265 ml. 1195 pounds of Resin A in the form of a 20.4% water solution were added to the refined pulp fiber and thoroughly mixed with it. At this point, 200 gallons of a 0.6% solution of a defoamer, and 30 pounds of aluminum sulfate which had been dissolved in a minimum amount of water were added. After these additions, the stock had a pH of 6.5 and a TAPPI freeness of 285 ml.

The stock was continuously pumped to the headbox of a cylinder papermachine, and a 2.5% water solution of Kymene 557 was metered into headbox at the rate of 1750 ml. per minute. After this point, recirculation of

white water from the cylinder vats resulted in a dilution of the stock to a consistency of between 0.42 and 0.49%. Immediately preceding the flow of the stock into the bottom of the cylinder vats, a 0.077% water solution of polyethylene oxide was metered into the stock at approximately 7500 ml. per minute. The stock was then dewatered on the cylinder mold, dried and machine calendered. A 25 point board having a basis weight of 93 pounds per thousand square feet was produced at a speed of 160 feet per minute. The composition of the board was 25.2% Resin A and 74.8% pulp fibers.

The board product was laminated to a 3 ply thickness with a heat setting adhesive. The laminated board when prestreamed for 60 seconds was easily formed in a press heated to a temperature of 160° F.

## EXAMPLE 22

400 grams of double kraft lined corrugated cuttings were dispersed in 20,000 ml. of water in a laboratory disintegrator and blended for a period of at least 60 minutes. The pulp stock was then reduced to 0.76% consistency and had a TAPPI freeness of 500 to 550 ml. To 95 ml. portions of the 0.76% pulp stock were added 286 ml. of a 3.0% Resin A solution, stirring the solution in slowly. Dilution water was added to give a subsequent total volume of 1188 ml., including all the desired additives. This corresponds to a resin-pulp consistency of approximately 0.8%. Additional ingredients were added in the following manner. The calcium chloride was added as 135 ml. of a 0.1 molar water solution of calcium chloride. Parez 607 was added as 9.5 ml. of a 0.1% water solution. The polyethylene oxide was added as 4.75 ml. of 0.1% polyethylene oxide in water. After each addition, the resin pulp stock was thoroughly mixed, avoiding excessive agitation, before the next ingredient was added.

After the polyethylene oxide was thoroughly mixed in, a handsheet containing approximately 90% resin was made in the manner described in Example 1. Resin retention was 98.6%.

The resin-filled board of the examples of this invention may be formed under heat and pressure into a wide variety of useful products. Luggage, automobile panels, trays, mannequins, containers and the like may be prepared simply and economically using shaped dies.

Having described the invention, it will be evident to those skilled in the art that the procedures described and the resultant products are adaptable to the use of any of a wide range of fibers. Chemical wood pulps and cellulosic fibers from other sources, inorganic fibers, both natural and manufactured, such as fibers from glass, asbestos fibers, synthetic organic fibers and the like may be used without departing from the scope of the invention.

Likewise, the product of the invention may be adapted to a wide range of uses by choice of resin, precipitating ion, amount of resin, density of the resin-fiber-board, and other obvious variations evident to those skilled in the art. Similarly, the surface of the resin-fiberboard of this invention may be treated with sizings and/or coatings to serve as a base for further decorative treatments. Finally, fibrous, relatively resin-free surface layers may be provided by employment of the process of the invention on the middle cylinders of a multi-cylinder machine while the liner cylinders operate on resin-free pulp stocks. For some uses, multiple layers of the resin-filled board can be assembled, as by pasting, to provide thicker sections as may be desired.

While the foregoing presents preferred embodiments of the present invention, it is obvious that other modifications and/or equivalents may be employed without departing from the scope of the invention, which is defined in the appended claims.

What is claimed is:

1. A new article of manufacture consisting essentially of a fibrous product having resinous material incorporated and substantially uniformly distributed therethrough, said product containing from about 15% to about 90% resinous material and from about 10% to about 85% fiber, said resinous material being present in the form of a polyvalent metal salt derived by the precipitation of the soluble alkali salt of the resinous material with a polyvalent metal ion, said fibrous product including a flocculant for said resinous material of about 0.002% to 0.1% high molecular weight polyethylene oxide based on the resin-fiber content.

2. A new article of manufacture consisting essentially of a fibrous product having resinous material incorporated and substantially uniformly distributed therethrough, said product containing from about 15% to about 90% resinous material and from about 10% to about 85% fiber, said resinous material being present in the form of a polyvalent metal salt derived by the precipitation of the soluble alkali salt of the resinous material with a polyvalent metal ion, said fibrous product including a flocculant for said resinous material of about 0.002% to 0.1% high molecular weight polyethylene oxide based on the resin-fiber content, said polyvalent metal ion being in the form of a water-soluble salt selected from the group consisting of calcium, barium, magnesium, strontium and aluminum and present in an amount up to three times the stoichiometric amount required.

3. A new article of manufacture consisting essentially of a fibrous product having resinous material incorporated and substantially uniformly distributed therethrough, said product containing from about 15% to about 90% resinous material and from about 10% to about 85% fiber, said resinous material being present in the form of a polyvalent metal salt derived by the precipitation of the soluble alkali salt of the resinous material with a polyvalent metal ion, said fibrous product including a flocculant for said resinous material of about 0.002% to 0.1% high molecular weight polyethylene oxide based on the resin-fiber content, said soluble alkali salt of the resinous material being selected from the group consisting of sodium salts of the acids present in tall oil and wood rosin; sodium salts of wood rosin, tall oil fatty acids, extracted pine wood pitch, abietic, oleic, stearic, linoleic acids; the ammonium salt of shellac and the sodium salt of alkali soluble polyvinyl acetate copolymers.

4. The fibrous product of claim 1 wherein the polyvalent metal ion is derived from calcium chloride.

5. The fibrous product of claim 1 wherein the polyvalent metal salt of the resinous material is derived from sodium salts of wood rosin.

6. The fibrous product of claim 1 wherein the polyvalent metal salt of the resinous material is derived from sodium salts of fatty acids.

7. The fibrous product of claim 1 wherein the resinous material consists essentially of an alkali soluble shellac.

8. The fibrous product of claim 1 wherein the resinous material consists essentially of alkali soluble polyvinyl acetate copolymers.

9. The fibrous product of claim 1 wherein the resinous material is a mixture of sodium salts of the acids present in tall oil and wood rosin in the ratio of 85% tall oil and 15% rosin.

10. A process for preparing a fibrous product containing from about 15% to about 90% resinous material and from about 10% to about 85% fiber which comprises the steps of preparing an aqueous dispersion of fibrous material with a polyvalent metal ion, said metal ion being in the form of a water-soluble salt selected from the group consisting of calcium, barium, magnesium, strontium and aluminum and present in an amount up to three times the stoichiometric amount required, treating the resulting fiber-metal ion solution with an alkali soluble

salt of a resinous material to precipitate said material in the form of a polyvalent metal salt, said alkali soluble salt of the resinous material being selected from the group consisting of sodium salts of the acids present in tall oil and wood rosin; sodium salts of wood rosin, tall oil fatty acids, extracted pine wood pitch, abietic acid, stearic, linoleic acids; the ammonium salt of shellac and the sodium salt of alkali soluble polyvinyl acetate copolymers, thereafter treating the resulting mixture with a solution of high molecular weight polyethylene oxide, the concentration of said polyethylene oxide being in the range of from 0.002% to 0.1% based on the resin-fiber content whereby said polyethylene oxide is capable of effecting the flocculation of said precipitated water soluble resinous material.

11. A process for preparing a fibrous product containing from about 15% to about 90% resinous material and from about 10% to about 85% fiber which comprises the steps of preparing an aqueous dispersion of fibrous material with a polyvalent metal ion, said metal ion being in the form of a water-soluble salt selected from the group consisting of calcium, barium, magnesium, strontium and aluminum and present in an amount up to three times the stoichiometric amount required, treating the resulting fiber-metal ion solution with a resinous material consisting essentially of a mixture of the sodium salts present in tall oil and wood rosin, in the ratio of 85% tall oil and 15% rosin, thereafter treating the resulting mixture with a solution of high molecular weight polyethylene oxide, the concentration of said polyethylene oxide being in the range of from 0.002% to 0.1% based on the resin-fiber content whereby said polyethylene oxide is capable of effecting the flocculation of said precipitated water soluble resinous material.

12. A process for preparing a fibrous product having a range of about 72.6% to substantially 100% resin retention, which comprises preparing an aqueous dispersion of fibrous material, interacting a polyvalent metal ion with a water soluble resinous material capable of being precipitated by a polyvalent metal ion, in intimate association with said dispersion of fibrous material, said polyvalent metal ion being in the form of a water-soluble salt selected from the group consisting of calcium, barium, magnesium, strontium and aluminum and present in an amount up to three times the stoichiometric amount required, thereafter treating the resulting mixture with a solution of high molecular weight polyethylene oxide whereby said polyethylene oxide is capable of effecting the flocculation of said precipitated water soluble resinous material.

13. A process for substantially uniformly dispersing resinous materials in a fibrous product comprising preparing a slurry of dispersed fibers, incorporating into said slurry with mild agitation a resinous material in the form of a polyvalent metal salt derived by the precipitation of the soluble alkali salt of the resinous material with a polyvalent metal ion, controlling the resulting floc size of said resinous material in the fibrous product by the introduction of a high molecular weight polyethylene oxide of a concentration of the order of 0.002% to 0.1% based in the resin-fiber content whereby said polyethylene oxide is capable of effecting the flocculation of said precipitated water soluble resinous material.

#### References Cited by the Examiner

#### UNITED STATES PATENTS

|           |         |                |       |         |
|-----------|---------|----------------|-------|---------|
| 1,840,399 | 1/1932  | Lane           | ----- | 162—179 |
| 2,447,064 | 8/1948  | Gebhart        | ----- | 162—179 |
| 2,712,994 | 7/1955  | Niles          | ----- | 162—179 |
| 2,987,489 | 6/1961  | Bailey et al.  | ----- | 260—2   |
| 3,008,868 | 11/1961 | Feigley et al. | ----- | 162—179 |
| 3,024,160 | 3/1962  | Kapral         | ----- | 162—179 |
| 3,112,242 | 11/1963 | Jones          | ----- | 162—180 |
| 3,141,815 | 7/1964  | Manley         | ----- | 162—164 |

(Other references on following page)

**15**

## FOREIGN PATENTS

498,054 12/1953 Canada.  
610,357 12/1960 Canada.

## OTHER REFERENCES

Bailey et al.: "High Molecular Weight Polymers of Ethylene Oxide," "Industrial and Engineering Chemistry," vol. 50, No. 1, January 1958, pp. 8-11.

**16**

"Development News," "Can You Profit by the Unique Properties of Pluronics?," vol. 30, No. 22, June 2, 1962, pp. 2283-2285.

5 DONALL H. SYLVESTER, *Primary Examiner.*  
S. L. BASHORE, *Examiner.*